

March 22, 1960

R. H. CARLSON

2,929,863

INSULATED OIL WELL CABLE

Filed Oct. 17, 1956



*Richard H. Carlson* INVENTOR  
By: *Donald S. Walton*  
his Attorney.

# United States Patent Office

2,929,863

Patented Mar. 22, 1960

1

2,929,863

## INSULATED OIL WELL CABLE

Richard H. Carlson, Boylston, Mass., assignor to United States Steel Corporation, a corporation of New Jersey

Application October 17, 1956, Serial No. 616,480

1 Claim. (Cl. 174—108)

This invention relates to an electric cable and an insulating composition used therein. The invention while applicable to various types of cable relates more particularly to a cable to be used in determining the characteristics of the strata at various levels in a deep oil well. Because of the conditions in deep oil wells, the insulating composition used must have certain characteristics which are present in prior used compositions which utilize natural rubber. However, in addition to these characteristics it is desirable that the weight and diameter of the cable be decreased as much as possible. The specific inductive capacity of insulating compositions used prior to my invention was relatively high, thus requiring a greater amount of insulation.

It is therefore an object of my invention to provide an oil well cable utilizing an insulating composition having a relatively low specific inductive capacity while retaining substantially the physical characteristics of the prior insulating compositions.

This and other objects would be more apparent after referring to the following specification and attached drawing, in which the single figure is a view of a well logging cable with parts broken away.

Referring more particularly to the drawings, reference numeral 2 indicates electrical conductors or strands each of which is made up of seven coated copper wires laid with a left hand lay. Insulating material 4 surrounds each of the conductors 2. It is this insulating material to which the present invention relates. The insulating material is extruded about each of the conductors in the usual manner. An electrical shielding compound 6 surrounds the insulating material 4 on each conductor 2. The purpose of the shielding composition is to overcome the electrostatic field between the conductors and to develop zero direct capacity. The shielding composition may be applied to the insulated strands either before or during the stranding of the insulated strands or conductors 2. The three covered conductors 2 are twisted together with a left hand lay and a filler material 8, such as glass, is laid in the interstices or valleys between the conductors 2. A binder 10 of cotton or similar material is helically wound about the conductors 2 and fillers 8 with a relatively long lay so as to hold these elements compactly together and to obtain a circular construction. Braid 12, such as white rayon, surrounds the binder 10. A layer of clear paraffin 14 may surround the rayon braid 12, if desired, and a semi-conducting shielding layer 16 surrounds the paraffin 14 or the braid 12 if no paraffin is used. The shielding layer 16 is of the same composition as the layer 6. A first layer of eighteen armor wires 18 surrounds the shielding compound and a second layer of eighteen armor wires 20 surrounds the first layer 18. The wires in the two layers are laid with opposite lay and it is preferred that the wires in the first layer be right lay and those in the second layer left lay. It will be understood that the number of conductors in the cable may vary, as many as seven conductors commonly being used.

The insulating composition of my invention includes 40 to 50 percent by weight of butadiene-styrene polymer in which there is approximately three times as much butadiene as styrene. The polymer may include slight amounts

2

of other materials such as a fraction of one percent of divinylbenzene. More than one type of polymer may be used as long as the ratio of butadiene-styrene does not vary more than a few percent. The composition also includes 12 to 16% by weight of a butadiene-styrene copolymer having approximately 15% (14% to 16%) butadiene and approximately 85% (84% to 86%) styrene, 0.6 to 1.0% by weight of a peptizer, 4 to 6% by weight of zinc oxide, 12 to 17% by weight of talc, 13 to 17% by weight of calcined clay, .50 to 1.5% by weight of an anti-oxidant, 1.0 to 2.0% by weight of paraffin wax, 0.30 to 0.70% by weight of fatty acid, 0.75 to 1.00% by weight of sulphur, 0.50 to 0.80% by weight of an accelerator, and 0.30 to 0.50% by weight of activator. A particular composition found to be suitable includes 29% of the composition GR-S-1019 and 16% of the composition GR-S-1018, these making up the butadiene-styrene polymer having approximately three times as much butadiene as styrene, 14% butadiene-styrene copolymer having 15% butadiene and 85% styrene, .88% naphthyl-beta mercaptan, this being the peptizer, 5% zinc oxide, 15.22% talc ground to 300 mesh or finer, 15% calcined clay, 1.00% 4 methyl-6-tertiary butyl phenol, this being the anti-oxidant, 1.50% paraffin wax, .50% stearic acid, 1.00% sulfur, .50% zinc dimethyl dithiocarbamate, this being the accelerator, and .40% mercaptobenzothiazole, this being the activator.

The butadiene-styrene polymers are the electrical grades of the polymers of butadiene and styrene which provide low water absorption because they have been treated to keep the water soluble ash and electrolyte at a minimum. The terms used above are well known in the art and are defined in the "Glossary of Terms Relating to Rubber and Rubber-Like Materials" published by the American Society for Testing Materials.

While one embodiment of my invention has been shown and described it will be apparent that other adaptations and modifications may be made without departing from the scope of the following claim.

I claim:

An oil well cable comprising a plurality of conductors twisted together, an insulating material surrounding each of said conductors, a filler in the valleys between the conductors, a binder surrounding said filler and conductors, and a layer of armor wires surrounding said binder, said insulating material consisting essentially of 40 to 50% by weight of butadiene-styrene copolymer in which there is approximately three times as much butadiene as styrene, 12 to 16% by weight of butadiene-styrene copolymer in which there is approximately 15% butadiene and 85% styrene, 0.6 to 1.00% by weight of peptizer, 4 to 6% by weight of zinc oxide, 12 to 17% by weight of talc, 13 to 17% by weight of calcined clay, 0.5 to 1.5% by weight of an anti-oxidant, 1.0 to 2.0% by weight of paraffin wax, 0.30 to 0.70% by weight of fatty acid, 0.75 to 1.00% by weight of sulphur, 0.50 to 0.80% by weight of accelerator, and 0.30 to 0.50% by weight of activator.

## References Cited in the file of this patent

### UNITED STATES PATENTS

|           |                |               |
|-----------|----------------|---------------|
| 2,234,068 | Wiseman        | Mar. 4, 1941  |
| 2,526,654 | Gleason et al. | Oct. 24, 1950 |
| 2,604,509 | Blanchard      | July 22, 1952 |
| 2,638,457 | Gates          | May 12, 1953  |
| 2,638,462 | Borders        | May 12, 1953  |

### FOREIGN PATENTS

|         |               |               |
|---------|---------------|---------------|
| 616,687 | Great Britain | Jan. 25, 1949 |
|---------|---------------|---------------|

### OTHER REFERENCES

The India-Rubber Journal, November 12, 1927, pages 897, 898.